

# UNITED STATES PATENT OFFICE.

CARL LUDWIG VALENTIN ZIMMER, OF BERLIN-WILMERSDORF, GERMANY, ASSIGNOR,  
BY MESNE ASSIGNMENTS, TO THE CHEMICAL FOUNDATION, INC., A CORPORATION  
OF DELAWARE.

## PROCESS FOR CONVERTING LIMESTONE INTO A COMPRESSIBLE ARTIFICIAL STONE.

1,391,710.

Specification of Letters Patent. Patented Sept. 27, 1921.

No Drawing. Original application filed August 11, 1915, Serial No. 45,023. Divided and this application filed February 7, 1918. Serial No. 215,940.

To all whom it may concern:

Be it known that I, CARL LUDWIG VALENTIN ZIMMER, doctor of philosophy, a subject of the King of Prussia, and a resident of Berlin-Wilmersdorf, Nos. 30-31 Pariserstrasse, Germany, have invented new and useful Improvements in Processes for Converting Limestone into a Compressible Artificial Stone, of which the following is a specification.

The present application is a division of my application, Serial No. 45023 filed August 11, 1915, for Letters Patent of the United States of America.

Heretofore no process was known for producing an artificial stone which has the property of decomposing to a powder when heated, and of regaining its original hardness under pressure.

Only natural asphaltic limestone, as found at but a few places on the earth in limited quantities, has the specially characteristic property that, when heated to 150-200° C., it decomposes to a brown, loose powder which can be compressed by pressure to the hardness of the original stone. Owing to these properties compressed asphalt, made from asphaltic limestone, is so extensively used for roads, and the like, since they satisfy all requirements in regard to resistance to mechanical stresses of all kinds, to frost and heat, etc.

Not every asphaltic limestone can be used directly for making roads, but only such sorts as contain 8-12% bitumen, whose melting point, moreover, is not higher than 50° C. (regulation of the road authorities). If both requirements are not satisfied, the compressed asphalt will not meet all demands of practice in regard to durability, softening point, etc. Since, even in one and the same mine, the amount of bitumen contained in the stone varies very much, it is extremely difficult to obtain a really good material.

The reason for the great advantages of compressed asphalt made from the natural product was considered to be due to the intimate mechanical mixture of the two components: limestone and bitumen. Various attempts have therefore been made to add bitumen to asphaltic limestone containing too little bitumen. Heat was also used to assist the operation, or bitumen was em-

ployed in the form of an emulsion. It is however not possible to obtain a good compressed asphalt by such means. The mass obtained has only the properties of cast asphalt, because according to the processes mentioned the bitumen was only brought into mechanical contact with the stone, or, in other words, only surrounds same. Further, all experiments made to mix powdered limestone or chalk with bitumen or other additions (compare *Chemical Technology* by Dr. H. Köhler, page 146) have not resulted in producing a compressible asphalt, but only a product having the properties of cast asphalt, that is, it melts when heated, and it cannot be compressed, when it solidifies. This nonsuccess was, in the first place, due to the fact that the chemical process, which unmistakably takes place between the bitumen and limestone in nature, was not recognized. Consequently, an expert came naturally to the conclusion that the artificial production of a stone, which, on being heated, decomposes to a loose powder, and can then be compressed, is quite impossible.

According to the present invention, it is rendered possible to produce a compressible asphalt synthetically, which not only in analysis and use shows the properties of natural asphaltic limestone, but even exceeds same by the fact that not only quantity of bitumen, but also the softening point of the bitumen can be chosen within the widest limits, and thus the most advantageous composition for any given purpose can be obtained.

In the endeavor to investigate, and, if, possible, to imitate, the operations which take place in the natural formation of asphaltic limestone, the inventor first ascertained that the formation of the natural product cannot have taken place in hot condition, because natural asphaltic limestone contains very low boiling hydrocarbons, which are essentially necessary to obtain the desired properties, and could not be present, if a higher temperature came into question. Further, it was recognized that the formation could not have taken place by bitumen being simply mixed with finely powdered limestone, but that rather a chemical process must have taken place. Considerations of this and other kinds, convinced the in-

ventor that the process in nature must have been of a chemical character.

Many experiments were made with the object of repeating this process artificially, 5 till finally the uniform presence of sulfur in natural asphaltic limestone led to the present process.

The material used for the purpose consists, on the one hand, as in the case of the 10 natural product, of limestone or any stone containing lime, such as calcareous spar, marble, chalk, etc.

The second material used, as in nature, is some bituminous substance, such as natural 15 asphalt, vegetable and animal oils, mineral oils, mineral oil residues, tar, tar oil residues and distillates.

If such bituminous substances, by means 20 of sulfated sebacic acid, or its alkaline salts, are converted into an emulsion, this emulsion, in a very dilute condition, will have the property, even at ordinary temperature, to quickly react on the powdered limestone, and will form an artificial asphaltic limestone 25 having all the properties set forth above, the attainment of which forms the object of the present application.

The chemical reaction, which takes place 30 between the sebacic acid and the powdered limestone, causes an intimate union of the limestone and bituminous substances to be effected.

For the purpose in question sulfo-acids 35 of animal and vegetable oil and fats, or their salts, are very suitable. Sulfated ricinoleic acids have been found to be of particular

advantage. When such are used the reaction is finished in a few minutes, and after mixing the materials the vessel must be quickly emptied, so quickly does the reaction take 40 place. The product obtained is at first an extremely plastic kneadable mass which decisively repels water.

The present process is, of course, an invention of the greatest importance. It is 45 not only suitable to entirely replace natural asphalt, but is even superior to such, inasmuch as this artificial asphaltic limestone, as above mentioned, affords the possibility of choosing in each case a composition suitable 50 for the particular conditions and temperature.

The term sebacic acid as used in the claims is intended as a generic term to include both the acid and its salts, precisely as when one speaks of a given amount of phosphoric acid 55 in a certain sample of soil.

What I claim and desire to secure by Letters Patent of the United States is:—

1. The herein described process of converting limestone into compressible artificial stone which consists in mixing stone containing lime with a bituminous substance containing sulfated sebacic acid. 60

2. The herein described process of converting limestone into compressible artificial stone which consists in mixing powdered limestone with a bituminous substance in the presence of sulfated sebacic acid capable of emulsifying the bituminous substance. 65

CARL LUDWIG VALENTIN ZIMMER.